

## UNITED STATES PATENT OFFICE

WILHELM ELLER, OF BERLIN-WILMERSDORF, AND RICHARD HOFSTADT, OF WOLFEN,  
KREIS BITTERFIELD, GERMANY, ASSIGNEES TO I. G. FARBENINDUSTRIE AKTIEN-  
GESELLSCHAFT, OF FRANKFORT-ON-THE-MAIN, GERMANY, A CORPORATION OF  
GERMANY

## MANUFACTURE OF ARTIFICIAL THREADS OR THE LIKE

No Drawing. Application filed May 31, 1929, Serial No. 367,612, and in Germany June 2, 1928.

The present invention relates to a new process of manufacturing artificial silk, threads, bands, horse hairs, films, etc. from viscose and to the new precipitating bath employed in this process.

It is based on the observation that halogenated fatty acids have a favorable influence on the operation of coagulating viscose. According to the invention halogenated fatty acids as for instance mono-, di-, tri-chloroacetic acid are added to the coagulating bath whereby products of good properties are obtained. For instance in the case of spinning artificial threads or bands from viscose, the presence of such acids in the bath lends to the products a tensile strength, extensibility, lustre and capacity for being dyed which suit all requirements.

The use of halogenated fatty acids is not associated with any particular bath. They may be used in any known bath provided, of course, that the bath does not react with halogenated fatty acids in an undesirable manner. For example, the spinning baths consisting of sulfuric acid and sulfuric acid salts in which artificial silk is commonly made may be mixed with one or more halogenated fatty acids. When departing from the usual spinning baths containing sulfuric acid and sodium sulfate, halogenated fatty acids may also be added without change of the bath but it may be advantageous to substitute the halogenated fatty acid for a more or less considerable portion of the mineral acid constituents of the spinning bath.

The nature of the halogenated fatty acid and the proportion which is added to the bath depend merely on the question of solubility. For example, the easily soluble monochloroacetic acid may be added in very considerable proportions in a quantity of for instance 10-30 per cent, whereas trichloroacetic acid is only slightly soluble in many of the usual baths. We prefer to add about 100 grams per liter of monochloroacetic acid to the precipitating bath, the quantity, however, depending on the other ingredients of the bath and the best results may be ascertained by a simple test. Obviously, we may use a mixture

of the halogenated fatty acids with the same effect.

The chief effect of the halogenated fatty acid in the bath is that it modifies the conditions of coagulation, for instance the speed of the action of the mineral acid is varied and thereby a product of good softness obtained. Moreover, by the use of such a spinning bath one is in the position to obtain under various conditions of maturity of viscose a fiber of constant good physical properties, such as tensile strength, pliability and lustre.

The action of the halogenated fatty acid can be considerably increased by using the acid in the form of an intermediate bath, through which the threads pass after they have left the spinning bath and before they are wound on the spools. The length of immersion in such an intermediate bath depends on the degree of concentration of the bath liquor.

With the action of halogenated fatty acids on forms of viscose as described above, there may be associated with special advantage a stretching of the form produced, for instance in spinning viscose to form artificial silk the addition of a halogenated fatty acid makes it possible to apply a very considerable tension to the thread, since the coagulating effect is diminished by the halogenated fatty acid and correspondingly the thread remains longer in a plastic condition when it has left the spinning nozzles than it does in baths which do not contain halogenated fatty acid.

The following examples illustrate the invention, which, however, is not limited to the specific details given therein:—

*Example 1.*—A viscose solution containing 7.5 per cent of cellulose and having a ripeness of  $4\frac{1}{4}$ , titrated with sodium chloride solution, is pressed through a nozzle with 60 openings of about 0.09 mm. diameter in a precipitating bath containing 13.5 per cent of sulfuric acid, 31 per cent of sodium sulfate and 55.5 per cent of water. The drawing speed is held at about 50 meters per minute, and the viscose pump delivers such a quantity of viscose that the bundle of threads obtained, has a titer of 120 deniers. The threads are stretched by guiding them over

glass rods. The temperature of this precipitating bath is kept at about 50° C. After having passed this precipitating bath, the threads are guided in a second bath containing 75 per cent of monochloracetic acid and 25 per cent of water, this second bath being kept at a temperature of 22° C. The threads obtainable in this manner have a tensile strength of about 250 grams per 100 deniers and an extensibility of about 8.5 per cent.

*Example 2.*—A viscose solution containing 7.5 per cent of cellulose and 7.5 per cent of alkali and having a normal ripeness, is spun into a precipitating bath containing 13.5 per cent of sulfuric acid, 31 per cent of sodium sulfate, 10 per cent of monochloracetic acid and 45.5 per cent of water. The threads may be stretched by guiding them on their way from the nozzle to the collection device over glass rods or through a suitable thread guide known in the art. The precipitating bath is kept at a temperature of about 50° C., the drawing speed may be maintained at about 50-60 meters per minute. The threads obtainable have a tensile strength of about 230 grams per 100 deniers and an extensibility of about 7-10 per cent.

*Example 3.*—A viscose solution is spun under the same conditions as mentioned in Example 2, the precipitating bath, however, contains instead of monochloracetic acid trichloracetic acid. Threads of similar qualities are obtained.

What we claim is:—

35 1. The process which comprises bringing viscose into the form of threads, bands, horsehairs, films and treating it in a bath containing a chlorinated fatty acid.

40 2. The process which comprises bringing viscose into the form of threads, bands, horsehairs, films and treating it in a bath containing monochloracetic acid.

45 3. Process for manufacturing artificial threads, bands, films or the like from a viscose solution which comprises pressing a viscose solution in a precipitating bath containing a halogenated fatty acid.

50 4. Process for manufacturing artificial threads, bands, films or the like from a viscose solution which comprises pressing a viscose solution in a precipitating bath containing sulfuric acid and a halogenated fatty acid.

55 5. Process for manufacturing artificial threads, bands, films or the like from a viscose solution which comprises pressing a viscose solution in a precipitating bath containing sulfuric acid, sodium sulfate and a halogenated fatty acid.

60 6. Process for manufacturing artificial threads, bands, films or the like from a viscose solution which comprises pressing a viscose solution in a precipitating bath containing sulfuric acid, sodium sulfate and a chlorinated acetic acid.

7. Process for manufacturing artificial threads, bands, films or the like from a viscose solution which comprises pressing a viscose solution in a precipitating bath containing sulfuric acid, sodium sulfate and monochloracetic acid. 70

8. A precipitating bath containing a chlorinated fatty acid and such products as are known in the art of spinning artificial fibers to be suitable to precipitate a viscose solution. 75

9. A precipitating bath containing sulfuric acid, sodium sulfate and monochloracetic acid.

10. Process for manufacturing artificial threads, bands, films or the like from a viscose solution which comprises pressing a viscose solution in a precipitating bath containing sulfuric acid, sodium sulfate and trichloracetic acid. 80

11. A precipitating bath containing sulfuric acid, sodium sulfate and trichloracetic acid. 85

In testimony whereof, we affix our signatures.

WILHELM ELLER.  
RICHARD HOFSTADT.

90

95

100

105

110

115

120

125

130